

## UNITED STATES PATENT OFFICE.

WALTER K. MARVIN, OF NEW YORK, N. Y.

## IMPROVED PLATES FOR CONSTRUCTING BURGLAR-PROOF SAFES, &amp;c.

Specification forming part of Letters Patent No. 41,629, dated February 16, 1864.

*To all whom it may concern:*

Be it known that I, WALTER K. MARVIN, of the city, county, and State of New York, have made a new and useful Improvement in the Construction of Burglar-Proof Safes; and I do hereby declare the following to be a full and clear description thereof.

My invention relates to the manufacture of iron sheets or plates which are impervious to drills employed under the conditions and provisions which are generally within the reach of and available to burglars, and the construction of the outer walls or case of fire and burglar proof safes with these prepared sheets or plates.

The means heretofore adopted for rendering the walls more difficult to drill or cut consist—

First. In employing three or more sheets of metal, the first being wrought-iron and the others steel and iron, alternately arranged.

Secondly. In casting Franklinit iron onto the face of a sheet of wrought-iron and placing this cast-iron facing against another sheet of wrought-iron, so that a thin stratum of Franklinit intervenes the two sheets of wrought-iron. The Franklinit iron is also sometimes cast into sheets and simply placed between the two wrought-iron sheets, instead of casting it onto one of the sheets, as above described. I may also mention that chilled cast-iron may be included in this class.

Thirdly. In the employment of various devices consisting of peculiar mechanical and architectural arrangements of parts—for instance, placing cast balls within the two sheets of iron, instead of a sheet of cast-steel, franklinit, or chilled iron—the object of these arrangements being that a drill penetrating the outer sheet and coming in contact with the balls will simply turn around with the ball and do no further harm, or, happening to strike between two balls or parts, would be wrenched and broken by the force employed to drive the drill. Other devices of this character have been suggested or used.

There are objections to each and all of these modes. The use of steel, as first named, involves great expense in the production of the walls, while it does not answer the purpose for which it is designed. The sheet-steel thus employed is known to the trade as "spring-steel." It is cut up into pieces of the required size and afterward tempered or hardened. Al-

though good spring-steel may be chosen for this purpose, yet it cannot be tempered so as to resist the action of a drill made of the best refined steel, which, being small and easily manageable, is tempered with great care and generally with superior skill. The second mode—that of employing franklinit—is much less perfect than that of steel. This is also true of chilled iron, as it is extremely brittle. Burglars have frequently overcome the apparent difficulty by cutting a disk from the outer sheet with a circular knife, and when the hard strata within are reached by fracturing the cast metal by a few blows of a hammer while the whole safe is muffled. The cast metal is thus made to crumble. The disk is then easily pried out, and no further obstacle is presented to the entrance of the safe. The last mode, which relates to the use of balls and such like mechanical arrangements, has proven in practice to be of little more utility in resisting the drill than would have been the case had the walls been of solid cast-iron, while safes made under such arrangements are generally expensive and bulky. Burglars have drilled through these walls with comparative ease by drilling through the outer sheet of metal and casting lead and sulphur through this aperture, so that the interior pieces or balls were cemented together, and therefore no more offered any obstruction to the further action of the drill. In some cases the interstices between the balls and other small pieces have been excellent receptacles of the gun-powder employed by the burglars for blasting. In other cases the burglars have simply cut a disk from the outer sheet of iron and then removed the balls or other internal contrivance calculated to deviate or break the tool, and they have then easily cut through the remaining sheets.

The object of my invention is to remedy difficulties, some of which I have designated, and I have accomplished it by the construction of walls or plates for safes and other purposes which cannot be drilled or cut by "circular knives."

To carry out this my invention I first take one of the ordinary rollers employed by iron-workers for rolling out sheet-iron. This is put on a planing-machining and corrugations or gutters of half-circle form are planed into its surface. The best effect has been obtained by me by forming equidistant grooves of about

O. 109-84

29/1/95, 163, 109-84, 109-84, 109-84

one-eighth of an inch wide and deep. This roller is replaced into the rolling-machine directly over a plain or smooth roller and adjusted at the required height above the other roller. A sheet of boiler-iron—say one-quarter of an inch thick—is now placed in a reverberatory furnace and heated to a rolling-heat. It is then taken out and passed through between the two rollers—*i. e.*, between the corrugated roller and the plain roller. The sheet will issue from the rollers corrugated on one side and plain-surfaced on the other, in conformity with the surfaces of the two rollers between which it was passed. The next step is to fill the gutters or depressions in the corrugated side of the sheet with granulated or powdered corundum or emery. This having been done, a second sheet of any desirable thickness, but of smooth or plain surface, is placed over the emery, and the two sheets are clamped or riveted together at the corners to prevent their displacement. The whole is now removed to the reverberatory furnace and heated to a welding-heat. It is next taking out and passed through the ordinary rolling-mill, consisting of pairs of smooth rollers. The result is that one solid sheet is obtained, which contains in its interior emery firmly embedded and held within an infinite number of little matrices of iron, while externally there are no indications denoting other than an ordinary sheet of iron.

I have described a sheet constructed by corrugating one of the two sheets of iron; but I have also, where heavy sheets have been desired, corrugated both sheets, and before placing the emery in the grooves I have riveted the two sheets together at the corners and cemented or sealed the ends of the tubes formed by bringing the two corrugated sides of the sheets together with a cement made of potter's clay and borax moistened a little with water. Then placing the sheets on edge, with the sealed end down, I filled the grooves with emery, and then closed the tubes on top with the cement. The whole is then put into the reverberatory furnace and heated to a welding-heat, and finally passed through the rolling-mill.

I have been more particular in describing these modes because I have obtained the best results from them; but I have obtained good results by punching holes of one-eighth of an inch in diameter over the surface of one or both the sheets to about one-half of their thickness, and by filling these with emery, and by otherwise proceeding as I have described in the other two modes.

A great number of practical and comparative trials of sheets made in the manner I have described as of my invention with sheets made according to modes heretofore practiced, some of which I have alluded to, have established the superior resistance of the emery sheets to

drills, circular knives, and other cutting-instruments. I have found that the effect of the emery on the best prepared drill is that of chipping off the edge in some instances and in others that of grinding away the cutting-edge of the drill. The peculiar hardness of the emery thus renders the drill useless.

In describing my invention I have confined myself thus far to the construction of safes; but it is obvious that it has other applications equally important. It may be applied to the construction of prison-bars and to other purposes where it is desirable that the iron should be impenetrable by saws, drills, and other cutting-instruments. It will likewise be understood that the particular form of grooves, gutters, or holes or depressions is not essential to the carrying out of my invention. I do not therefore desire to confine myself to the particular forms or modes which I have described as most convenient or readily practicable in carrying out my invention. Nor do I wish to be understood as limiting myself to the use of wrought-iron plates exclusively, as emery may be combined with steel or cast-iron; but when applied to the latter, owing to the brittleness of cast metals, the advantages due to my invention could be easily counteracted.

Having thus described my invention and the manner in which the same is or may be carried into effect, I would state my claims as follows:

1. As a new composition of matter, iron or steel combined with emery, substantially in the manner and for the purposes set forth.
2. Combining emery with malleable iron or steel by rolling process, as set forth.
3. The manufacture of plates or sheets of iron or steel by welding together two or more plates or sheets having emery interposed, substantially as herein set forth.
4. The method of making iron or steel plates having an emery core or emery confined in cells throughout the interior, as described, by forming the same of two or more plates, either or all of which are corrugated, grooved, or have depressions or recesses formed therein for containing and holding the emery during the welding and rolling operations, as set forth.

5. The manufacture of burglar-proof safes, prison-bars, and other objects calculated to resist the action of cutting or piercing instruments of iron or steel, made in the manner hereinbefore described.

In testimony whereof I have signed my name to this specification before two subscribing witnesses.

WALTER K. MARVIN.

Witnesses:

JAMES M. RAYMOND,  
EDWARD BISSELL.